

A. H. REID.

BRAKE SHOE.

APPLICATION FILED APR. 26, 1916.

1,205,482.

Patented Nov. 21, 1916.

FIG. 1.



FIG. 2.



FIG. 3.



WITNESSES:

A. V. Walsh  
M. E. Critchley

INVENTOR

Andrew H. Reid.

BY

George Cook, Esq.  
ATTORNEYS.

# UNITED STATES PATENT OFFICE.

ANDREW H. REID, OF TORONTO, ONTARIO, CANADA, ASSIGNOR TO AMERICAN BRAKE SHOE & FOUNDRY COMPANY, OF MAHWAH, NEW JERSEY, A CORPORATION OF NEW JERSEY.

## BRAKE-SHOE.

1,205,482.

Specification of Letters Patent. Patented Nov. 21, 1916.

Application filed April 26, 1916. Serial No. 93,580.

To all whom it may concern:

Be it known that I, ANDREW H. REID, a subject of His Majesty, the King of Great Britain, and a resident of Toronto, Province of Ontario, Canada, have made and invented certain new and useful Improvements in Brake-Shoes, of which the following is a specification.

My object is to devise a cheap strong 10 brake shoe which will have high braking efficiency combined with long life.

I attain my object by means of a construction which may be briefly described as follows: On a suitable metal back is cast a shoe 15 of hydraulic cement suitably reinforced with metal and bound to the back. The cement has added thereto various ingredients intended to improve its frictional qualities.

A suitable construction for the shoe is 20 illustrated in the accompanying drawings, in which:—

Figure 1 is a longitudinal section of a brake shoe constructed in accordance with my invention; Fig. 2, a cross section; and 25 Fig. 3 a plan view of the face of the shoe.

In the drawings, like letters of reference indicate corresponding parts in the different figures.

A is a back preferably of steel provided 30 with the attaching lugs B.

In molding the shoe I secure in suitable positions relative to the back a plurality of layers of metallic reinforcement C, preferably of a reticulated form such as expanded metal. The cement body D of the shoe is then cast about the back and reinforcement. The layers of reinforcing metal may run in any desired direction through the body of the shoe as may be found desirable 40 and part of the reinforcement is preferably carried around the back to bind the body of the shoe thereto. The ends E of the back may be turned down into the body of the shoe, and tubes F may be supported 45 therein which run through the shoe, as in my prior U. S. Patent No. 943,995, and Canadian Patent No. 122,502. These tubes serve to lighten and strengthen the shoe, but are not indispensable in the present construction.

While a good hydraulic cement, such as Portland cement, will give useful results, I find that the best results are obtained when

some friction increasing substance is added to the cement. For this purpose I employ 55 sulfur, preferably in a proportion not exceeding 30 parts of sulfur to 70 of cement. The sulfur may be in part replaced by metallic antimony, salt, and asbestos, mica or crushed iron ore. I do not, however, desire 60 to confine myself to the use of any specific friction increasing ingredients, as others than those specified may be found useful for my purposes.

A shoe such as described will be found to 65 satisfactorily attain the objects of my invention, as the reinforced concrete is light and strong, and its surface does not burn off as does the surface of iron and steel shoes. I further find that the reticulated metal so 70 binds together every part of the body of the shoe that it has no more tendency to split or crack than any good all metal shoe.

What I claim as my invention is:—

1. A brake shoe comprising a tough metal 75 back; a plurality of layers of reticulated metal and a body of hydraulic cement cast about said back and reinforcement and binding the same together.

2. A brake shoe formed of a mixture of 80 hydraulic cement and sulfur reinforced with metal.

3. A brake shoe formed of a mixture of 85 hydraulic cement, sulfur and salt, reinforced with metal.

4. A brake shoe formed of a mixture of 90 hydraulic cement, sulfur, salt and antimony reinforced with metal.

5. A brake shoe formed of a mixture of 95 hydraulic cement, sulfur, salt, antimony and asbestos reinforced with metal.

6. A brake shoe comprising a tough metal back; a plurality of layers of reticulated metal in part inclosing said back and a body of hydraulic cement cast about said back 95 and reinforcement and binding the same together.

Signed at New York, borough of Manhattan, in the county of New York and State of New York, this 18th day of April, A. D. 100 1916.

ANDREW H. REID.

Witnesses:

ANNA V. WALSH,  
GEORGE E. COOK.